# EUROPEAN PATENT SPECIFICATION

(11) **EP 0 422 019 B1**
(45) Date of publication and mention of the grant of the patent: **01.12.1993**
(21) Application number: 89905983.6
(22) Date of filing: 28.04.1989
(51) Int. Cl.: C10M 107/10, C08F 10/14, C07C 9/22, C08F 4/24, C10N 20/00

(54) **OLEFINIC OLIGOMERS HAVING LUBRICATING PROPERTIES AND PROCESS OF MAKING SUCH OLIGOMERS**
OLEFINOLIGOMERE MIT SCHMIERUNGSEIGENSCHAFTEN UND VERFAHREN ZU IHRER HERSTELLUNG
OLIGOMERES OLEFINIQUES AYANT DES PROPRIETES LUBRIFIANTES ET LEUR PROCEDE DE PRODUCTION

(30) Priority: 23.06.1988 US 210434; 23.06.1988 US 210435
(43) Date of publication of application: 17.04.1991
(73) Proprietor: MOBIL OIL CORPORATION, New York New York 10017 (US)
(72) Inventor: WU, Margaret, May-Som, Belle Mead, NJ 08502 (US)
(74) Representative: Colmer, Stephen Gary
(86) International application number: US8901843
(87) International publication number: WO8912662

(56) References cited:
- EP-A- 0 000 748
- EP-A- 0 034 303
- DE-A- 3 427 319
- US-A- 3 206 523
- US-A- 4 282 392
- US-A- 4 362 654
- US-A- 4 587 368

## Description

This invention relates to novel lubricant compositions and more particularly, to novel synthetic lubricant compositions prepared from alpha-olefins, or 1-alkenes. The invention specifically relates to novel synthetic lubricant compositions from 1-alkenes exhibiting superior viscosity indices and other improved characteristics essential to useful lubricating oils. This invention further relates to a process for manufacturing such lubricant compositions.

Efforts to improve upon the performance of natural mineral oil based lubricants by the synthesis of oligomeric hydrocarbon fluids have been the subject of important research and development in the petroleum industry for at least fifty years and have led to the relatively recent market introduction of a number of superior polyalpha-olefin (PAO) synthetic lubricants, primarily based on the oligomerization of alpha-olefins or 1-alkenes. In terms of lubricant property improvement, the thrust of the industrial research effort on synthetic lubricants has been toward fluids exhibiting useful viscosities over a wide range of temperature, i.e., improved viscosity index (VI), while also showing lubricity, thermal and oxidative stability and pour point equal to or better than mineral oil. These new synthetic lubricants lower friction and hence increase mechanical efficiency across the full spectrum of mechanical loads from worm gears to traction drives and do so over a wider range of operating conditions than mineral oil lubricants.

The chemical focus of the research effort in synthetic lubricants has been on the polymerization of 1-alkenes. Well known structure/property relationships for high polymers as contained in the various disciplines of polymer chemistry have pointed the way to 1-alkenes as a fruitful field of investigation for the synthesis of oligomers with the structure thought to be needed to confer improved lubricant properties thereon. Due largely to studies on the polymerization of propene and vinyl monomers, the mechanism of the polymerization of 1-alkene and the effect of that mechanism on polymer structure is reasonably well understood, providing a strong resource for targeting on potentially useful oligomerization methods and oligomer structures. Building on that resource, in the prior art oligomers of 1-alkenes from C₆ to C₂₀ have been prepared with commercially useful synthetic lubricants from 1-decene oligomerization yielding a distinctly superior lubricant product via either cationic or Ziegler catalyzed polymerization.

Theoretically, the oligomerization of 1-decene, for example, to lubricant oligomers in the C₃₀ and C₄₀ range can result in a very large number of structural isomers. Henze and Blair,J.A.C.S. 54,1538, calculate over 60 x10¹² isomers for C₃₀-C₄₀. Discovering exactly those isomers, and the associated oligomerization process, that produce a preferred and superior synthetic lubricant meeting the specification requirements of wide-temperature fluidity while maintaining low pour point represents a prodigious challenge to the workers in the field. Brennan, Ind. Eng. Chem. Prod. Res. Dev. 1980, 19, 2-6, cites 1-decene trimer as an example of a structure compatible with structures associated with superior low temperature fluidity wherein the concentration of atoms is very close to the center of a chain of carbon atoms. Also described therein is the apparent dependency of properties of the oligomer on the oligomerization process, i.e., cationic polymerization or Ziegler-type catalyst, known and practiced in the art.

One characteristic of the molecular structure of 1-alkene oligomers that has been found to correlate very well with improved lubricant properties in commercial synthetic lubricants is the ratio of methyl to methylene groups in the oligomer. The ratio is called the branch ratio and is calculated from infra red data as discussed in "Standard Hydrocarbons of High Molecular Weight", Analytical Chemistry, Vol.25, no. 10, p.1466 (1953). Viscosity index has been found to increase with lower branch ratio. Heretofore, oligomeric liquid lubricants exhibiting very low branch ratios have not been synthesized from 1-alkenes. For instance, oligomers prepared from 1-decene by either cationic polymerization or Ziegler catalyst polymerization have branch ratios of greater than 0.20. Shubkin, Ind. Eng.Chem. Prod. Res. Dev. 1980, 19, 15-19, provides an explanation for the apparently limiting value for branch ratio based on a cationic polymerization reaction mechanism involving rearrangement to produce branching. Other explanations suggest isomerization of the olefinic group in the one position to produce an internal olefin as the cause for branching. Whether by rearrangement, isomerization or a yet to be elucidated mechanism it is clear that in the art of 1-alkene oligomerization to produce synthetic lubricants as practiced to-date excessive branching occurs and constrains the limits of achievable lubricant properties, particularly with respect to viscosity index. Obviously, increased branching increases the number of isomers in the oligomer mixture, orienting the composition away from the structure which would be preferred from a consideration of the theoretical concepts discussed above.

US-A-4,282,392 to Cupples et al. discloses an alpha-olefin oligomer synthetic lubricant having an improved viscosity-volatility relationship and containing a high proportion of tetramer and pentamer via a hydrogenation process that effects skeletal rearrangement and isomeric composition. The composition claimed is a trimer to tetramer ratio no higher than one to one. The branch ratio is not disclosed.

US-A-3 206 523 discloses compositions which differs from those of the invention in that the branch ratio is higher than 0.16.

A process using coordination catalysts to prepare high polymers from 1-alkenes, especially chromium catalyst on a silica support, is described by Weiss et al. in Jour. Catalysis 88, 424-430 (1984) and in DE-A-3,427,319. The process and products therefrom are discussed in more detail hereinafter in comparison with the process and products of the instant invention.

It is well known that Lewis acids such as promoted BF₃ and/or metal halides can catalyze Friedel-Crafts type reactions. However, olefin oligomers and more particularly PAO oligomers have been produced by methods in which double bond isomerization of the starting 1-olefin occurrs easily. As a result, the olefin oligomers have more short side branches. These side branches degrade their lubricating properties.

Liquid hydrocarbon lubricant compositions have been obtained from C₆-C₂₀, preferably C₈-C₁₂, 1-alkene oligomerization that exhibit surprisingly high viscosity index (VI) while, equally surprisingly, exhibit very low pour points. The compositions comprise C₃₀-C₁₃₀₀ hydrocarbons, the compositions having a branch ratio of between 0.1 and 0.16; weight average molecular weight between 300 and 45,000; number average molecular weight between 300 and 18,000; molecular weight distribution between 1 and 5 and pour point below -15°C. The hydrocarbons comprise alkanes or alkenes. The compositions have a viscosity index greater than 130 and viscosity at 100°C between 3mm²/s and 750 mm²/s.

Further, a novel composition has been discovered comprising 11-octyldocosane having the structure

The foregoing composition has been found to exhibit superior lubricant properties either alone or in a mixture with 9-methyl,11-octylheneicosane. Surprisingly, the mixture has a viscosity index of greater than 130, preferably from 130 to 280, while maintaining a pour point less than -15°C. These compositions are representative of the instant invention comprising C₃₀H₆₂ alkanes having a branch ratio, or CH₃/CH₂ ratio, of between 0.10 and 0.16. These low branch ratios and pour points characterize the compositions of the invention, referred to herein as polyalpha-olefin or HVI-PAO, conferring upon the compositions especially high viscosity indices in comparison to commercially available polyalpha-olefin (PAO) synthetic lubricants.

Unique lubricant oligomers of the instant invention an also be made in a wide range of molecular weights and viscosities comprising C₃₀ to C₁₀₀₀ hydrocarbons having a branch ratio of between 0.10 and 0.16 and molecular weight distribution of about 1.05 to 2.5. The oligomers can be mixed with conventional mineral oils or greases of other properties to provide compositions also possessing outstanding lubricant properties.

Compositions of the present invention comprise the polymeric residue of 1 alkenes taken from linear C₆-C₂₀, preferably C₈-C₁₂, alkenes and can be prepared by the oligomerization of alpha-olefins such as 1-decene under oligomerization conditions in contact with a supported and reduced valence state metal oxide catalyst from Group VIB of the IUPAC Periodic Table. Chromium oxide is the preferred metal oxide. Optionally, the composition can be hydrogenated. Preferably, the polymeric residue comprises poly 1-decene having a molecular weight of about 422, a viscosity index of about 134 and a pour point of less than -45°C.

The present invention provides a process for producing liquid oligomers of olefins, such as 1-decene, with branch ratios of between 0.10 and 0.16 and having higher viscosity indices than oligomers with higher branch ratios. These oligomers with low branch ratios can be used as basestocks for many lubricants or greases with an improved viscosity-temperature relationship, oxidative stability, volatility, etc. They can also be used to improve viscosities and viscosity indices of lower quality oils. The olefins can, for example, be oligomerized over a supported and reduced metal oxide catalyst from Group VIB of the Periodic Table to give oligomers suitable for lubricant application. More particularly, the instant application is directed to a process for the oligomerization of olefinic hydrocarbons containing 6 to 20 carbon atoms which comprises oligomerizing said hydrocarbon under oligomerization conditions, wherein the reaction product consists essentially of substantially non-isomerized olefins. Oligomerization conditions comprise a temperature of 90°C to 250°C, preferably 100°C to 180°C, with a chromium catalyst on a porous support which catlyst has been treated by oxidation at a temperature of 200°C to 900°C in the presence of an oxidizing gas and then by treatment with a reducing agent, such as CO, at a temperature and for sufficient time to reduce the catalyst to a lower valence state. For example, alpha olefins such as 1-decene, and wherein a major proportion of the double bonds of the olefins or olefinic hydrocarbons are not isomerized, in the presence of a suitable catalyst, e.g., a supported and reduced metal oxide catalyst from Group VIB of the Periodic Table. The yield of the C₃₀+ oligomer is at least 85 wt% for product having a viscosity of at least 15 mm²/s at 100°C. The catalyst is not subjected to a further oxidation step after the reduction. In a preferred embodiment, the olefin comprises 1-decene and the oligomer has a VI of 181 or greater and a branch ratio of 0.14 to 0.16.

The use of reduced Group VIB chromium-containing metal oxide on an inert support oligomerizes liquid olefins which are suitable for use as good quality lube oils is a novel technique.

Figure 1 is a comparison of PAO and HVI-PAO syntheses.

Figure 2 compares VI for PAO and HVI-PAO

Figure 3 shows pour points for PAO and HVI-PAO

Figure 4 shows C-13 NMR spectra for HVI-PAO from 1-hexene.

Figure 5 shows C-13 NMR spectra of 5 mm²/s HVI-PAO from 1-decene.

Figure 6 shows C-13 NMR spectra of 50 mm²/s HVI-PAO from 1-decene.

Figure 7 shows C-13 NMR spectra of 145 mm²/s HVI-PAO from 1-decene.

Figure 8 shows the gas chromatograph of HVI-PAO 1-decene trimer.

Figure 9 shows C-13 NMR of HVI-PAO trimer of 1-decene.

Figure 10 shows C-13 NMR calculated vs. observed chemical shifts for HVI-PAO 1-decene trimer components.

In the following description, unless otherwise stated, all references to HVI-PAO oligomers or lubricants refer to hydrogenated oligomers and lubricants in keeping with the practice well known to those skilled in the art of lubricant production. As oligomerized, HVI-PAO oligomers are mixtures of dialkyl vinyledenic and 1,2 dialkyl or trialkyl mono-olefins. Lower molecular weight unsaturated oligomers are preferably hydrogenated to produce thermally and oxidatively stable, useful lubricants. Higher molecular weight unsaturated HVI-PAO oligomers are sufficiently thermally stable to be utilized without hydrogenation and, optionally, may be so employed. Both unsaturated and hydrogenated HVI-PAO of lower or higher molecular exhibit viscosity indices of at least 130, preferably from 130 to 280, and pour point below -15°C, preferably -45°C.

Referring to Figure 1, the novel oligomers of the invention, or high viscosity index polyalphaolefins (HVI-PAO) are described in an illustration comparing them with conventional polyalphaolefins (PAO) from 1-decene. Polymerization with the novel reduced chromium catalyst described hereinafter leads to an oligomer substantially free of double bond isomerization. Conventional PAO, on the other hand, promoted by BF₃ or AlCl3 forms a carbonium ion which, in turn, promotes isomerization of the olefinic bond and the formation of multiple isomers. The HVI-PAO produced in the present invention has a structure with a CH₃/CH₂ ratio<0.19 compared to a ratio of >0.20 for PAO.

Figure 2 compares the viscosity index versus viscosity relationship for HVI-PAO and PAO lubricants, showing that HVI-PAO is distinctly superior to PAO at all viscosities tested. Remarkably, despite the more regular structure of the HVI-PAO oligomers as shown by branch ratio that results in improved viscosity index (VI), they show pour points superior to PAO. Conceivably, oligomers of regular structure containing fewer isomers would be expected to have higher solidification temperatures and higher pour points, reducing their utility as lubricants. But, surprisingly, such is not the case for HVI-PAO of the present invention. Figure 2 and 3 illustrate superiority of HVI-PAO in terms of both pour point and VI.

It has been found that the process described herein to produce the novel HVI-PAO oligomers can be controlled to yield oligomers having weight average molecular weight between 300 and 45,000 and number average molecular weight between 300 and 18,000. Measured in carbon numbers, molecular weights range from C₃₀ to C₁₃₀₀ and viscosity up to 750 mm²/s(cs) at 100°C, with a preferred range of C₃₀ to C₁₀₀₀ and a viscosity of up to 5000 mm²/s(cs) at 100°C, preferably between 3 and 750 mm²/s. Molecular weight distributions (MWD), defined as the ratio of weight average molecular weight to number average molecular weight, range from 1.00 to 5, with a preferred range of 1.01 to 3 and a more preferred MWD of about 1.05 to 2.5. Compared to conventional PAO derived from BF₃ or AlCl₃ catalyzed polymerization of 1-alkene, HVI-PAO of the present invention has been found to have a higher proportion of higher molecular weight polymer molecules in the product.

Viscosities of the novel HVI-PAO oligomers measured at 100°C range from 3 mm²s(cs) to 5000 mm²/s(cs). The viscosity index for the new polyalpha-olefins is approximately described by the following equation:
${\text{VI =129.8 + 4.58 x (V₁₀₀°C)}}^{\text{0.5}}$ , where V₁₀₀ C is kinematic viscosity in centistokes measured at 100°C.

The novel oligomer compositions disclosed herein have been examined to define their unique structure beyond the important characteristics of branch ratio and molecular weight already noted. Dimer and trimer fractions have been separated by distillation and components thereof further separated by gas chromatography. These lower oligomers and components along with complete reaction mixtures of HVI-PAO oligomers have been studied using infra-red spectroscopy and C-13 NMR. The studies have confirmed the highly uniform structural composition of the products of the invention, particularly when compared to conventional polyalphaolefins produced by BF₃, AlCl₃ or Ziegler-type catalysis. The unique capability of C -13 NMR to identify structural isomers has led to the identification of distinctive compounds in lower oligomeric fractions and served to confirm the more uniform isomeric mix present in higher molecular weight oligomers compatible with the finding of low branch ratios and superior viscosity indices.

1-hexene HVI-PAO oligomers of the present invention have been shown to have a very uniform linear C₄ branch and contain regular head-to-tail connections. In addition to the structures from the regular head-to-tail connections, the backbone structures have some head-to-head connection, indicative of the following structure as confirmed by NMR:
The NMR poly(1-hexene) spectra are shown in Figure 4.

The oligomerization of 1-decene by reduced valence state, supported chromium also yields a HVI-PAO with a structure analogous to that of 1-hexene oligomer. The lubricant products after distillation to remove light fractions and hydrogenation have characteristic C-13 NMR spectra. Figures 5, 6 and 7 are the C-13 NMR spectra of typical HVI-PAO lube products with viscosities of 5 mm²/s(cs), 50 mm²/s(cs) and 145 mm²/s(cs) at 100°C.

In the following tables, Table A presents the NMR data for Figure 5, Table B presents the NMR data for Figure 6 and Table C presents the NMR data for Figure 7.

**Table A**

| (Fig. 5) | | | |
|---|---|---|---|
| Point | Shift(ppm) | Intensity | Width(Hz) |
| 1 | 79.096 | 138841. | 2.74 |
| 2 | 74.855 | 130653. | 4.52 |
| 3 | 42.394 | 148620. | 6.68 |
| 4 | 40.639 | 133441. | 37.6 |
| 5 | 40.298 | 163678. | 32.4 |
| 6 | 40.054 | 176339. | 31.2 |
| 7 | 39.420 | 134904. | 37.4 |
| 8 | 37.714 | 445452. | 7.38 |
| 9 | 37.373 | 227254. | 157 |
| 10 | 37.081 | 145467. | 186 |
| 11 | 36.788 | 153096. | 184 |
| 12 | 36.593 | 145681. | 186 |
| 13 | 36.447 | 132292. | 189 |
| 14 | 36.057 | 152778. | 184 |
| 15 | 35.619 | 206141. | 184 |
| 16 | 35.082 | 505413. | 26.8 |
| 17 | 34.351 | 741424. | 14.3 |
| 18 | 34.059 | 1265077. | 7.65 |
| 19 | 32.207 | 5351568. | 1.48 |
| 20 | 30.403 | 3563751. | 4.34 |
| 21 | 29.965 | 8294773. | 2.56 |
| 22 | 29.623 | 4714955. | 3.67 |
| 23 | 28.356 | 369728. | 10.4 |
| 24 | 28.161 | 305878. | 13.2 |
| 25 | 26.991 | 1481260. | 4.88 |
| 26 | 22.897 | 4548162. | 1.76 |
| 27 | 20.265 | 227694. | 1.99 |
| 28 | 14.221 | 4592991. | 1.62 |

**Table B**

| (Fig. 6) | | | |
|---|---|---|---|
| No. | Freq(Hz) | PPM | Int% |
| 1 | 1198.98 | 79.147 | 1856 |
| 2 | 1157.95 | 77.004 | 1040 |
| 3 | 1126.46 | 74.910 | 1025 |
| 4 | 559.57 | 37.211 | 491 |
| 5 | 526.61 | 35.019 | 805 |
| 6 | 514.89 | 34.240 | 1298 |
| 7 | 509.76 | 33.899 | 1140 |
| 8 | 491.45 | 32.681 | 897 |
| 9 | 482.66 | 32.097 | 9279 |
| 10 | 456.29 | 30.344 | 4972 |
| 11 | 488.24 | 29.808 | 9711 |
| 12 | 444.58 | 29.564 | 7463 |
| 13 | 426.26 | 28.347 | 1025 |
| 14 | 401.36 | 26.691 | 1690 |
| 15 | 342.77 | 22.794 | 9782 |
| 16 | 212.40 | 14.124 | 8634 |
| 17 | 0.00 | 0.000 | 315 |

**Table C**

| (Fig. 7) | | | |
|---|---|---|---|
| Point | Shift(ppm) | Intensity | Width(Hz) |
| 1 | 76.903 | 627426. | 2.92 |
| 2 | 40.811 | 901505. | 22.8 |
| 3 | 40.568 | 865686. | 23.1 |
| 4 | 40.324 | 823178. | 19.5 |
| 5 | 37.158 | 677621. | 183. |
| 6 | 36.915 | 705894. | 181. |
| 7 | 36.720 | 669037. | 183. |
| 8 | 36.428 | 691870. | 183. |
| 9 | 36.233 | 696323. | 181. |
| 10 | 35.259 | 1315574. | 155. |
| 11 | 35.015 | 1471226. | 152. |
| 12 | 34.333 | 1901096. | 121. |
| 13 | 32.726 | 1990364. | 120. |
| 14 | 32.141 | 20319110. | 2.81 |
| 15 | 31.362 | 661594. | 148. |
| 16 | 30.388 | 9516199. | 19.6 |
| 17 | 29.901 | 17778892. | 9.64 |
| 18 | 29.609 | 18706236. | 9.17 |
| 19 | 28.391 | 869681. | 122. |
| 20 | 27.514 | 1117864. | 173. |
| 21 | 26.735 | 954012. | 14.0 |
| 22 | 22.839 | 20895526. | 2.17 |
| 23 | 14.169 | 16670130. | 2.06 |

In general, the novel oligomers have the following regular head-to-tail structure where n can be 3 to 17, x is 5 to 500:
with some head-to-head connections.
Preferably, n is 7 and average x is at least 15. The oligomers have a viscosity index greater than 130 and a pour point less than -15°C.

The trimer of 1-decene HVI-PAO oligomer is separated from the oligomerization mixture by distillation from a 20 mm²/s(cs) as-synthesized HVI-PAO in a short-path apparatus in the range of 165-210°C at 13.3-26.6 Pa (0.1-0.2 torr). The unhydrogenated trimer exhibited the following viscometric properties:
V @ 40°C = 14.88 mm²/s(cs); V @ 100°C = 3.67 mm²/s(cs); VI = 137
The trimer is hydrogenated at 235°C and 4200 kPa H₂ with Ni on kieselguhr hydrogenation catalyst to give a hydrogenated HVI-PAO trimer with the following properties:
V @ = 40°C = 16.66 mm²/s(cs); V @ 100°C = 3.91 mm²/s(cs) VI = 133
Pour Point = less than -45°C;
Gas chromatographic analysis of the trimer reveals that it is composed of essentially two components having retention times of 1810 seconds and 1878 seconds under the following conditions:
Gas chromatograph (g.c.) column-60 meter capillary column, 0.32 mmid (mm inside diameter), coated with stationary phase SPB-1 with film thickness 0.25mm, available from Supelco chromatography supplies, catalog no. 2-4046.

Separation Conditions - Varian Gas chromatograph, model no. 3700, equipped with a flame ionization detector and capillary injector port with split ratio of about 50. N₂ carrier gas flow rate is 2.5 ml/minute. Injector port temperature 300°C; detector port temperature 330°C, column temperature is set initially at 45°C for 6 minutes, programmed heating at 15°C/minute to 300°C final temperature and holding at final temperature for 60 minutes. Sample injection size is 1 microliter. Under these conditions, the retention time of a g.c. standard, n-dodecane, is 968 seconds.

A typical chromatograph is shown in Figure 8.

The C-13 NMR spectra, (Figure 9), of the distilled C30 product confirm the chemical structures. Table D lists C-13 NMR data for Figure 9.

**Table D**

| (Fig. (9) | | | |
|---|---|---|---|
| Point | Shift(ppm) | Intensity | Width(Hz) |
| 1 | 55.987 | 11080. | 2.30 |
| 2 | 42.632 | 13367. | 140. |
| 3 | 42.388 | 16612. | 263. |
| 4 | 37.807 | 40273. | 5.90 |
| 5 | 37.319 | 12257. | 16.2 |
| 6 | 36.539 | 11374. | 12.1 |
| 7 | 35.418 | 11631. | 35.3 |
| 8 | 35.126 | 33099. | 3.14 |
| 9 | 34.638 | 39277. | 14.6 |
| 10 | 34.054 | 110899. | 3.32 |
| 11 | 33.615 | 12544. | 34.9 |
| 12 | 33.469 | 13698. | 34.2 |
| 13 | 32.981 | 11278. | 5.69 |
| 14 | 32.835 | 13785. | 57.4 |
| 15 | 32.201 | 256181. | 1.41 |
| 16 | 31.811 | 17867. | 24.6 |
| 17 | 31.470 | 13327. | 57.4 |
| 18 | 30.398 | 261859. | 3.36 |
| 19 | 29.959 | 543993. | 1.89 |
| 20 | 29.618 | 317314. | 1.19 |
| 21 | 28.838 | 11325. | 15.1 |
| 22 | 28.351 | 24926. | 12.4 |
| 23 | 28.156 | 29663. | 6.17 |
| 24 | 27.230 | 44024. | 11.7 |
| 25 | 26.986 | 125437. | -0.261 |
| 26 | 22.892 | 271278. | 1.15 |
| 27 | 20.260 | 17578. | -22.1 |
| 28 | 14.167 | 201979. | 2.01 |

The individual peak assignment of the C-13 spectra are shown in Figure 9. Based on these structures, the calculated chemical shifts, as shown in Figure 10, matched closely with the observed chemical shifts. The calculation of chemical shifts of hydrocarbons is carried out as described is "Carbon-13 NMR for Organic Chemists" by G. C. Levy and G. L. Nelson, 1972, by John Wiley & Sons, Inc., Chapter 3, p 38-41. The components were identified as 9-methyl,11-octylheneicosane and 11- octyldocosane by infra-red and C-13 NMR analysis and were found to be present in a ratio between 1:10 and 10:1, preferably between 1:2 and 2:1, heneicosane to docosane. The hydrogenated 1-decene trimer produced by the process of this invention has an index of refraction at 60°C of 1.4396.

The process of the present invention produces a surprisingly simpler and useful dimer compared to the dimer produced by 1-alkene oligomerization with BF₃ or AlCl₃ as commercially practiced. Typically, in the present invention it has been found that a significant proportion of unhydrogenated dimerized 1-alkene has a vinylidenyl structure as follows:

CH₂=CR₁R₂

where R₁ and R₂ are alkyl groups representing the residue from the head-to-tail addition of 1-alkene molecules. For example, 1-decene dimer of the invention has been found to contain only three major components, as determined by GC. Based on C¹³ NMR analysis, the unhydrogenated components were found to be 8-eicosene, 9-eicosene, 2-octyldodecene and 9-methyl-8 or 9-methyl-9-nonadecene. The hydrogenated dimer components were found to be n-eicosane and 9-methylnonacosane.

Olefins suitable for use as starting material in the invention include those olefins containing from 2 to about 20 carbon atoms such as ethylene, propylene, 1-butene, 1-pentene, 1-hexene, 1-octene, 1-decene, 1-dodecene and 1-tetradecene and branched chain isomers such as 4-methyl-1-pentene. Also suitable for use are olefin-containing refinery feedstocks or effluents. However, the olefins used in this invention are preferably alpha olefinic as for example 1-heptene to 1-hexadecene and more preferably 1-octene to 1-tetradecene, or mixtures of such olefins.

Oligomers of alpha-olefins in accordance with the invention have a low branch ratio of between 0.1 and 0.16 and superior lubricating properties compared to the alpha-olefin oligomers with a high branch ratio, as produced in all known commercial methods.

This new class of alpha-olefin oligomers are prepared by oligomerization reactions in which a major proportion of the double bonds of the alphaolefins are not isomerized. These reactions include alpha-olefin oligomerization by supported metal oxide catalysts, such as Cr compounds on silica or other supported IUPAC Periodic Table Group VIB compounds. The catalyst most preferred is a lower valence Group VIB metal oxide on an inert support. Preferred supports include silica, alumina, titania, silica alumina, magnesia and the like. The support material binds the metal oxide catalyst. Those porous substrates having a pore opening of at least 40 x 10⁻⁴ µm are preferred.

The support material usually has high surface area and large pore volumes with average pore size of 40 to 350 x 10⁻⁴ µm. The high surface area are beneficial for supporting large amount of highly dispersive, active chromium metal centers and to give maximum efficiency of metal usage, resulting in very high activity catalyst. The support should have large average pore openings of at least 40 x 10⁻⁴ µm, with an average pore opening of 60 to 300 x 10⁻⁴ µm being preferred. This large pore opening will not impose any diffusional restriction of the reactant and product to and away from the active catalytic metal centers, thus further optimizing the catalyst productivity. Also, for this catalyst to be used in fixed bed or slurry reactor and to be recycled and regenerated many times, a silica support with good physical strength is preferred to prevent catalyst particle attrition or disintegration during handling or reaction.

The supported metal oxide catalysts are preferably prepared by impregnating metal salts in water or organic solvents onto the support. Any suitable organic solvent known to the art may be used, for example, ethanol,methanol, or acetic acid. The solid catalyst precursor is then dried and calcined at 200 to 900°C by air or other oxygen-containing gas. Thereafter the catalyst is reduced by any of several various and well known reducing agents such as, for example, CO, H₂, NH₃, H₂S, CS₂, CH₃SCH₃, CH₃SSCH₃,metal alkyl containing compounds such as R₃Al, R₃B,R₂Mg, RLi, R₂Zn, where R is alkyl, alkoxy, aryl and the like. Preferred are CO or H₂ or metal alkyl containing compounds.

Alternatively, the Group VIB metal may be applied to the substrate in reduced form, such as CrII compounds. The resultant catalyst is very active for oligomerizing olefins at a temperature range from below room temperature to about 250°C, preferably 90°-250°C, most preferably 100°- 180°C, at a pressure of 10.1 kPa (0.1 atmosphere) to 34500 kPa (5000 psi). Contact time of both the olefin and the catalyst can vary from one second to 24 hours. The weight hourly space velocity (WHSV) is 0.1 to 10, based on total catalyst weight. The catalyst can be used in a batch type reactor or in a fixed bed, continuous-flow reactor.

In general the support material may be added to a solution of the metal compounds, e.g., acetates or nitrates, etc., and the mixture is then mixed and dried at room temperature. The dry solid gel is purged at successively higher temperatures to 600°C for a period of 16 to 20 hours. Thereafter the catalyst is cooled down under an inert atmosphere to a temperature of 250 to 450°C and a stream of pure reducing agent is contacted therewith for a period when enough CO has passed through to reduce the catalyst as indicated by a distinct color change from bright orange to pale blue. Typically, the catalyst is treated with an amount of CO equivalent to a two-fold stoichiometric excess to reduce the catalyst to a lower valence CrII state.Finally the catalyst is cooled down to room temperature and is ready for use.

The product oligomers have a very wide range of viscosities with high viscosity indices suitable for high performance lubrication use. The product oligomers also have atactic molecular structure of mostly uniform head-to-tail connections with some head-to-head type connections in the structure. These low branch ratio oligomers have high viscosity indices at least 15 to 20 units and typically 30-40 units higher than equivalent viscosity prior art oligomers, which regularly have higher branch ratios and correspondingly lower viscosity indices. These low branch oligomers maintain better or comparable pour points.

The branch ratios defined as the ratios of CH₃ groups to CH₂ groups in the lube oil are calculated from the weight fractions of methyl groups obtained by infrared methods, published in Analytical Chemistry, Vol. 25, No. 10, p. 1466 (1953).
As referenced hereinbefore, supported Cr metal oxide in different oxidation states is known to polymerize alpha olefins from C₃ to C₂₀ (De 3427319 to H. L. Krauss and Journal of Catalysis 88, 424-430, 1984) using a catalyst prepared by CrO₃ on silica. The referenced disclosures teach that polymerization takes place at low temperature, usually less than 100 °C, to give adhesive polymers and that at high temperature, the catalyst promotes isomerization, cracking and hydrogen transfer reactions. The present inventions produce low molecular weight oligomeric products under reaction conditions and using catalysts which minimize side reactions such as 1-olefin isomerization, cracking, hydrogen transfer and aromatization. To produce the novel low molecular weight products suitable for use as lube basestock or as blending stock with other lube stock, the reaction of the present invention is carried out at a temperature higher (90-250 oC) than the temperature suitable to produce high molecular weight polyalpha-olefins. The catalysts used in the present invention do not cause a significant amount of side reactions even at high temperature when oligomeric, low molecular weight fluids are produced.

The catalysts for this invention thus minimize all side reactions but oligomerize alpha olefins to give low molecular weight polymers with high efficiency. It is well known in the prior art that chromium oxides, especially chromia with average +3 oxidation states, either pure or supported, catalyze double bond isomerization, dehydrogenation, cracking, etc. Although the exact nature of the supported Cr oxide is difficult to determine, it is thought that the catalyst of the present invention is rich in Cr(II) supported on silica, which is more active to catalyze alpha-olefin oligomerization at high reaction temperature without causing significant amounts of isomerization, cracking or hydrogenation reactions, etc. However, catalysts as prepared in the cited references can be richer in Cr (III). They catalyze alpha-olefin polymerization at low reaction temperature to produce high molecular weight polymers. However, as the references teach, undesirable isomerization, cracking and hydrogenation reaction takes place at higher temperatures. In contrast, high temperatures are needed in this invention to produce lubricant products. The prior art also teaches that supported Cr catalysts rich in Cr(III) or higher oxidation states catalyze 1-butene isomerization with 10³ higher activity than polymerization of 1-butene. The quality of the catalyst, method of preparation, treatments and reaction conditions are critical to the catalyst performance and composition of the product produced and distinguish the present invention over the prior art.

In the instant invention very low catalyst concentrations based on feed, from 10 wt%, to 0.01 wt%, are used to produce oligomers; whereas, in the cited references catalyst ratios based on feed of 1:1 are used to prepare high polymer. Resorting to lower catalyst concentrations in the present invention to produce lower molecular weight material runs counter to conventional polymerization theory, compared to the results in the cited references.

The oligomers of 1-olefins prepared in this invention usually have much lower molecular weights than the polymers produced in cited reference which are semi-solids, with very high molecular weights. These high polymers are not suitable as lubricant basestocks and usually have no detectable amount of dimer or trimmer (C₁₀-C₃₀) components form synthesis. Such high polymers also have very low unsaturations. However, products in this invention are free-flowing liquids at room temperature, suitable for lube basestock, containing significant amount of dimer or trimer and have high unsaturations.

### Example 1

### Catalyst Preparation and Activation Procedure

1.9 grams of chromium (II) acetate (Cr₂(OCOCH₃)₄2H₂O)(5.58 mmole) (commercially obtained) is dissolved in 50 ml of hot acetic acid. Then 50 grams of a silica gel of 8-12 mesh size, a surface area of 300 m²/g, and a pore volume of 1 ml/g, also is added. Most of the solution is absorbed by the silica gel. The final mixture is mixed for half an hour on a rotavap at room temperature and dried in an open-dish at room temperature. First, the dry solid (20 g) is purged with N₂ at 250°C in a tube furnace. The furnace temperature is then raised to 400°C for 2 hours. The temperature is then set at 600°C with dry air purging for 16 hours. At this time the catalyst is cooled down under N₂ to a temperature of 300°C. Then a stream of pure CO (99.99% from Matheson) is introduced for one hour. Finally, the catalyst is cooled down to room temperature under N₂ and ready for use.

### Example 2

The catalyst prepared in Example 1 (3.2 g ) is packed in a 3/8" (0.95 cm) stainless steel tubular reactor inside an N₂ blanketed dry box. The reactor under N₂ atmosphere is then heated to 150°C by a single-zone Lindberg furnace. Pre-purified 1-hexene is pumped into the reactor at 965 kPa (140 psi) and 20 ml/hr. The liquid effluent is collected and stripped of the unreacted starting material and the low boiling material at 6.7 kPa (0.05 mm Hg). The residual clear, colorless liquid has viscosities and VI's suitable as a lubricant base stock.

### Example 3

Similar to Example 2, a fresh catalyst sample is charged into the reactor and 1-hexene is pumped to the reactor at 101 kPa (1 atm) and 10 ml per hour. As shown below, a lube of high viscosities and high VI's is obtained. These runs show that at different reaction conditions, a lube product of high viscosities can be obtained.

### Example 4

A commercial chrome/silica catalyst which contains 1% Cr on a large-pore volume synthetic silica gel is used. The catalyst is first calcined with air at 800°C for 16 hours and reduced with CO at 300°C for 1.5 hours. Then 3.5 g of the catalyst is packed into a tubular reactor and heated to 100°C under the N₂ atmosphere. 1-Hexene is pumped through at 28 ml per hour at 101 kPa (1 atmosphere). The products are collected and analyzed as follows:

These runs show that different Cr on a silica catalyst are also effective for oligomerizing olefins to lube products.

### Example 5

As in Example 4, purified 1-decene is pumped through the reactor at 1830 kPa to 2310 kPa (250 to 320 psi). The product is collected periodically and stripped of light products boiling points below 343°C (650°F). High quality lubes with high VI are obtained (see following table).

| Reaction Temp.°C | WHSV g/g/hr | Lube Product Properties | | |
|---|---|---|---|---|
| | | V at 40°C (mm²/s) | V at 100°C (mm²/s) | VI |
| 120 | 2.5 | 1555.4 | 157.6 | 217 |
| 135 | 0.6 | 389.4 | 53.0 | 202 |
| 150 | 1.2 | 266.8 | 36.2 | 185 |
| 166 | 0.6 | 67.7 | 12.3 | 181 |
| 197 | 0.5 | 21.6 | 5.1 | 172 |

### Example 6

Similar catalyst is used in testing 1-hexene oligomerization at different temperature. 1-Hexene is fed at 28 ml/hr and at 101 kPa (1 atmosphere).

### Example 7

1.5 grams of a similar catalyst as prepared in Example 4 was added to a two-neck flask under N₂ atmosphere. Then 25 g of 1-hexene was added. The slurry was heated to 55°C under N₂ atmosphere for 2 hours. Then some heptane solvent was added and the catalyst was removed by filtration. The solvent and unreacted starting material was stripped off to give a viscous liquid with a 61% yield. This viscous liquid had viscosities of 1536 and 51821 mm²/2 (cs) at 100°C and 40°C, respectively. This example demonstrated that the reaction can be carried out in a batch operation.

The 1-decene oligomers as described below were synthesized by reacting purified 1-decene with an activated chromium on silica catalyst. The activated catalyst was prepared by calcining chromium acetate (1 or 3% Cr) on silica gel at 500-800°C for 16 hours, followed by treating the catalyst with CO at 300-350°C for 1 hour. 1-Decene was mixed with the activated catalyst and heated to reaction temperature for 16-21 hours. The catalyst was then removed and the viscous product was distilled to remove low boiling components at 200°C/13.3 kPa(0.1 mmHg).

Reaction conditions and results for the lube synthesis of HVI-PAO are summarized below:

**Table 1**

| Example NO. | Cr on Silica | Calcination Temp. | Treatment Temp. | 1-decene/Catalyst Ratio | Lube Yld |
|---|---|---|---|---|---|
| 8 | 3wt% | 700°C | 350°C | 40 | 90 |
| 9 | 3 | 700 | 350 | 40 | 90 |
| 10 | 1 | 500 | 350 | 45 | 86 |
| 11 | 1 | 600 | 350 | 16 | 92 |

### Branch Ratios and Lube Properties of Examples 8-11 Alpha Olefin Oligomers

**Table 2**

| Example No. | Branch CH₃ Ratios CH₂ | V40°C mm²/s | V100°C mm²/s | VI |
|---|---|---|---|---|
| 8 | 0.14 | 150.5 | 22.8 | 181 |
| 9 | 0.15 | 301.4 | 40.1 | 186 |
| 10 | 0.16 | 1205.9 | 128.3 | 212 |
| 11 | 0.15 | 5238.0 | 483.1 | 271 |

### Branch Ratios and Lubricating Properties of Alpha Olefin Oligomers Prepared in the Prior-Art

**Table 3**

| Example No. | Branch CH₃ Ratios CH₂ | V40°C mm²/s | V100°C mm²/s | VI |
|---|---|---|---|---|
| 12 | 0.24 | 28.9 | 5.21 | 136 |
| 13 | 0.19 | 424.6 | 41.5 | 148 |
| 14 | 0.19 | 1250 | 100 | 168 |
| 15 | 0.19 | 1247.4 | 98.8 | 166 |

These samples are obtained from the commercial market. They have higher branch ratios than samples in Table 2. Also, they have lower VI's than the previous samples.

Comparison of these two sets of lubricants clearly demonstrates that oligomers of alpha-olefins, as 1-decene, with branch ratios lower than 0.19, preferably from 0.13 to 0.18, have higher VI and are better lubricants. The examples prepared in accordance with this invention have branch ratios of 0.14 to 0.16, providing lube oils of excellent quality which have a wide range of viscosities from 3 to 483.1 mm²/s at 100°C with viscosity indices of 130 to 280.

### Example 16

A commercial Cr on silica catalyst which contains 1% Cr on a large pore volume synthetic silica gel is used. The catalyst is first calcined with air at 700°C for 16 hours and reduced with CO at 350°C for one to two hours. 1.0 part by weight of the activated catalyst is added to 1-decene of 200 parts by weight in a suitable reactor and heated to 185°C. 1-Decene is continuously fed to the reactor at 2-3.5 parts/minute and 0.5 parts by weight of catalyst is added for every 100 parts of 1-decene feed. After 1200 parts of 1-decene and 6 parts of catalyst are charged, the slurry is stirred for 8 hours. The catalyst is filtered and light product boiled below 150°C @ 0.1mm Hg is stripped. The residual product is hydrogenated with a Ni on Kieselguhr catalyst at 200°C. The finished product has a viscosity at 100°C of 18.5 mm²/s(cs), VI of 165 and pour point of -55°C.

### Example 17

Similar as in Example 16, except reaction temperature is 125°C. The finished product has a viscosity at 100°C of 145 mm²/s(cs), VI of 214, pour point of -40°C.

### Example 18

Example 16 is repeated except reaction temperature is 100°C. The finished product has a viscosity at 100°C of 298 mm²/s, VI of 246 and pour point of -32°C.

The final lube products in Example 16 to 18 contain the following amounts of dimer and trimer and isomeric distribution (distr.).

These three examples demonstrate that the new HVI-PAO of wide viscosities contain the dimer and trimer of unique structures in various proportions.

The molecular weights and molecular weight distributions are analyzed by a high pressure liquid chromatography, composed of a Constametric II high pressure, dual piston pump from Milton Roy Co. and a Tracor 945 LC detector. During analysis, the system pressure is 4600 kPa (650 psi) and THF solvent (HPLC grade) deliver rate is 1 ml per minute. The detector block temperature is set at 145 °C. ml of sample, prepared by dissolving 1 gram PAO sample in ml THF solvent, is injected into the chromatograph. The sample is eluted over the following columns in series,all from Waters Associates: Utrastyragel 10⁵ A, P/N 10574, Utrastyragel 10⁴ A, P/N 10573, Utrastyragel 10³ A, P/N 10572, Utrastyragel 500 A, P/N 10571. The molecular weights are calibrated against commercially available PAO from Mobil Chemical Co, Mobil SHF-61 and SHF-81 and SHF-401.

The following table summarizes the molecular weights and distributions of Examples 16 to 18.

| Examples | 16 | 17 | 18 |
|---|---|---|---|
| V @100 °C,mm²/s(cs) | 18.5 | 145 | 298 |
| VI | 165 | 214 | 246 |
| number-averaged molecular weights, MWₙ | 1670 | 2062 | 5990 |
| weight-averaged molecular weights, MW₌w | 2420 | 4411 | 13290 |
| molecular weight distribution, MWD | 1.45 | 2.14 | 2.22 |

Under similar conditions, HVI-PAO product with viscosity as low as 3 mm²/s (cs) and as high as 500 mm²/s (cs), with VI between 130 and 280, can be produced.

Ethene can be employed as a starting material for conversion to higher C₆-C₂₀ alpha olefins by conventional catalytic procedure, for instance by contacting ethene with a Ni catalyst at 80-120°C and about 7000 kPa (1000 psi) using commercial synthesis methods described in Chem System Process Evaluation/Research Planning Report - Alpha-Olefins, report number 82-4. The intermediate product alpha olefin has a wide distribution range from C₆ to C₂₀ carbons. The complete range of alpha olefins from growth reaction, or partial range such as C₆ to C₁₄, can be used to produce a lube of high yields and high viscosity indices. The oligomers after hydrogenation have low pour points.

### Example 19

An alpha olefin growth reaction mixture, as described above, containing C₆-C₈-C₁₀-C₁₂-C₁₄-C₁₆-C₁₈-C₂₀ of equal molar concentration is reacted with 2 wt. % activated Cr/SiO₂ catalyst at 130°C and under nitrogen atmosphere. After 225 minutes reaction time, the catalyst is filtered and the reaction mixture distilled to remove light fraction which boils below 120°C/0.1 mm-Hg. The residual lube yield is 95% and has V_{100°C} 67.07 mm²/s and VI 195.

### Example 20

An equimolar C₆-C₂₀ alpha olefin mixture as described above is fed continuously over activated Cr/SiO₂ catalyst packed in a tubular reactor. The results are summarized below.

### Example 21

Equimolar olefin mixture of C₆-C₈-C₁₀-C₁₂-C₁₄ is reacted over Cr/SiO₂ catalyst similar to Example 2. The results are summarized in Table 21.

A range of alpha olefins from ethylene growth reactions and metathesis processes can be used to produce high quality lube by the present process, thus rendering the process cheaper and the feedstock flexible than using pure single monomer.

### Example 22

The standard 1-decene oligomerization synthesis procedure employed above is repeated at 125°C using different Group VIB metal species, tungsten or molydenum. The W/Mo treated porous substrate is reduced with CO at 460°C to provide 1 wt. % metal in reduced oxide state. Molybdenum catalyst gives a 1% yield of a viscous liquid. Tungsten gives C₂₀ dimer only.

The use of supported Group VIB oxides as a catalyst to oligomerize olefins to produce low branch ratio lube products with low pour points was heretofore unknown. Catalytic production of low branch ratio which does not use a corrosive co-catalyst and produces a lube with a wide range of viscosities and good V.I.'s was also heretofore unknown and more specifically the preparation of lube oils having a branch ratio of between 0.1 and 0.16 was also unknown heretofore.

## Claims

1. A liquid lubricant composition comprising C₃₀-C₁₃₀₀ hydrocarbons, said composition having a branch ratio of between 0.1 and 0.16, weight average molecular weight between 300 and 45,000, number average molecular weight between 300 and 18,000, molecular weight distribution between 1 and 5 and pour point below -15°C.

2. The composition of claim 1 wherein said hydrocarbons comprise C₃₀-C₁₀₀₀ hydrocarbons and molecular weight distribution of 1.05 to 2.5.

3. The composition of claim 1 wherein said hydrocarbons comprise alkanes or alkenes.

4. The composition of claim 1 having a viscosity index greater than 130 and viscosity at 100°C between 3 mm²/s and 750 mm²/s..

5. The composition of claim 1 having a C₃₀ fraction with viscosity index greater than 130 and a pour point below -45°C.

6. The composition of claim 1 wherein the composition comprises the polymeric residue of 1-alkenes taken from linear C₆ - C₂₀ 1-alkenes.

7. The composition of claim 6 wherein said 1-alkenes comprise C₈-C₁₂ alkenes.

8. The composition of claim 6 wherein said polymeric residue comprises hydrogenated polymeric residue of said 1-alkenes.

9. The composition of claim 6 wherein said polymeric residue comprises poly 1-decene.

10. The composition of claim 9 wherein the polymeric residue of 1-decene has a molecular weight of about 422.

11. The composition of claim 10 having a viscosity index of about 134 and a pour point less than -45°C.

12. A liquid lubricant hydrocarbon composition having the recurring polymeric structure where n is 3 to 17 and x is 5 to 500.

13. The composition of claim 12 where n is seven and average x is at least fifteen.

14. The composition of claim 12 having a viscosity index greater than 130 and a pour point less than -15°C.

15. The hydrocarbon composition of any one of the preceding claims wherein the C₃₀-C₁₃₀₀ hydrocarbons comprise 9-methyl, 11-octylheneicosane and 11-octyldocosane.

16. The composition of claim 15 wherein the mole ratio of 9-methyl, 11-octylheneicosane:11-octyldocosane is between 1:10 and 10:1.

17. The composition of claim 16 wherein said mole ratio is preferably 1:2 to 2:1.

18. The composition of claim 15 wherein the 11-octyldocosane has the structure,

19. A process fo the preparation of liquid hydrocarrbons suitable as lubricant basestocks from alpha olefins containing 6 to 20 carbon atoms, or mixtures of such olefins, comprising: contacting said olefins under oligomerization conditions, at reaction temperature of about 90 to 250°C with a chromium catalyst on a porous support, which catalyst has been treated by oxidation at a temperature of 200°C to 900°C in the presence of an oxidizing gas and then by treatment with a reducing agent at a temperature and for a time sufficient to reduce said catalyst to a lower valence state; to obtain an oligomeric liquid lubricant composition comprising C₃₀-C₁₃₀₀ hydrocarbons, said composition having a branch ratio between 0.1 and 0.16, weight average molecular weight between 300 and 45,000, number average molecular weight between 300 and 18,000, molecular weight distribution between 1 and 5 and a pour point below -15°C.

20. The process of claim 19 wherein said reducing agent comprises CO, the oligomerization temperature is about 100-180°C, and the yield of C₃₀+ oligomer is at least 85 wt% for product having a viscosity of at least 15 mm²/s at 100°C.

21. The process of claim 19 or 20 wherein the support comprises porous silica.

22. The process of claim 19, 20 or 21 wherein the olefin consists essentially of 1-octene, 1-decene, 1-dodecene, 1-tetradecene or mixtures thereof.

23. The process of claim 19, 20, or 21 wherein said catalyst is not subjected to a further oxidation step after said reduction.

24. The process of claim 19, 20, or 21 wherein said olefin comprises 1-decene, and the oligomer has a VI of 181 or greater and a branch ratio of from 0.14 to 0.16.

## Patentansprüche

1. Flüssige Schmiermittelzusammensetzung, die C₃₀-C₁₃₀₀-Kohlenwasserstoffe umfaßt, wobei die Zusammensetzung ein Verzweigungsverhältnis zwischen 0,1 und 0,16, ein gewichtsmittleres Molekulargewicht zwischen 300 und 45000, ein zahlenmittleres Molarkulargewicht zwischen 300 und 18000, eine Molekulargewichtsverteilung zwischen 1 und 5 und einen Fließpunkt unterhalb von -15°C aufweist.

2. Zusammensetzung nach Anspruch 1, worin die Kohlenwasserstoffe C₃₀-C₁₀₀₀-Kohlenwasserstoffe und eine Molekulargewichtsverteilung von 1,05 bis 2,5 umfassen.

3. Zusammensetzung nach Anspruch 1, worin die Kohlenwasserstoffe Alkane oder Alkene umfassen.

4. Zusammensetzung nach Anspruch 1, die einen Viskositätsindex von mehr als 130 und bei 100°C eine Viskosität zwischen 3 mm²/s und 750 mm²/s aufweist.

5. Zusammensetzung nach Anspruch 1, mit einer C₃₀-Fraktion mit einem Viskositätsindex von mehr als 130 und einem Fließpunkt unterhalb von -45°C.

6. Zusammensetzung nach Anspruch 1, worin die Zusammensetzung den Polymerrückstand der 1-Alkene, der aus linearen C₆-C₂₀ 1-Alkenen stammt, umfaßt.

7. Zusammensetzung nach Anspruch 6, worin die 1-Alkene C₈-C₁₂ Alkene umfassen.

8. Zusammensetzung nach Anspruch 6, worin der Polymerrückstand den hydrierten Polymerrückstand der 1-Alkene umfaßt.

9. Zusammensetzung nach Anspruch 6, worin der Polymerrückstand Poly-1-Decen umfaßt.

10. Zusammensetzung nach Anspruch 9, worin der Polymerrückstand aus 1-Decen ein Molekulargewicht von etwa 422 aufweist.

11. Zusammensetzung nach Anspruch 10 mit einem Viskositätsindex von etwa 134 und einem Fließpunkt von weniger als -45°C.

12. Flüssige Schmiermittel-Kohlenwasserstoffzusammensetzung mit der wiederkehrenden Polymerstruktur worin n 3 bis 17 ist und x 5 bis 500 ist.

13. Zusammensetzung nach Anspruch 12, worin n sieben und das durchschnittliche x mindestens fünfzehn beträgt.

14. Zusammensetzung nach Anspruch 12 mit einem Viskositätsindex von mehr als 30 und einem Fließpunkt von weniger als -15°C.

15. Kohlenwasserstoffzusammensetzungen nach einem der vorangegangenen Ansprüche, worin die C₃₀-C₁₃₀₀-Kohlenwasserstoffe 9-Methyl-11-octylheneicosan und 11-Octyldocosan umfassen.

16. Zusammensetzung nach Anspruch 15, worin das Molverhältnis von 9-Methyl-11-Octylheneicosan:11-Octyldocosan zwischen 1:10 und 10:1 beträgt.

17. Zusammensetzung nach Anspruch 16, worin das Molverhältnis vorzugsweise 1:2 bis 2:1 beträgt.

18. Zusammensetzung nach Anspruch 15, worin das 11-Octyldocosan die Struktur aufweist.

19. Verfahren zur Herstellung flüssiger Kohlenwasserstoffe, die als Schmiermittelgrundmaterialien geeignet sind, aus Alphaolefinen, die 6 bis 20 Kohlenstoffatome enthalten, oder aus Gemischen solcher Olefine, das umfaßt: Kontaktierung der Olefine unter Oligomerisierungsbedingungen bei einer Reaktionstemperatur von etwa 90 bis 250°C mit einem Chromkatalysator an einem porösen Träger, wobei dieser Katalysator durch Oxidation bei einer Temperatur von 200°C bis 900°C in Gegenwart eines oxidierenden Gases und dann mit einem Reduktionsmittel bei einer Temperatur und für eine zur Reduktion des Katalysators in eine niedrige Wertigkeitsstufe ausreichende Zeit behandelt wurde, um eine oligomere, flüssige Schmiermittelzusammensetzung zu erhalten, die C₃₀-C₁₃₀₀-Kohlenwasserstoffe umfaßt, wobei die Zusammensetzung ein Verzweigungsverhältnis zwischen 0,1 und 0,16, ein gewichtsmittleres Molekulargewicht zwischen 300 und 45000, ein zahlenmittleres Molekulargewicht zwischen 300 und 18000, eine Molekulargewichtsverteilung zwischen 1 und 5 und einen Fließpunkt unterhalb von -15°C aufweist.

20. Verfahren nach Anspruch 19, worin das Reduktionsmittel CO umfaßt, die Oligomerisierungstemperatur etwa 100-180°C beträgt und die Ausbeute an C₃₀-Oligomer für ein Produkt mit einer Viskosität von mindestens 15 mm²/s bei 100°C mindestens 85 Gew.-% beträgt.

21. Verfahren nach Anspruch 19 oder 20, worin der Träger poröses Siliciumdioxid umfaßt.

22. Verfahren nach Anspruch 19, 20 oder 21, worin das Olefin im wesentlichen aus 1-Octen, 1-Decen, 1-Dodecen, 1-Tetradecen oder aus Gemischen daraus besteht.

23. Verfahren nach Anspruch 19, 20 oder 21, worin der Katalysator nach der Reduktion keiner weiteren Oxidation unterworfen wird.

24. Verfahren nach Anspruch 19, 20 oder 21, worin das Olefin 1-Decen umfaßt und das Oligomer einen VI von 181 oder größer und ein Verzweigungsverhältnis von 0,14 bis 0,16 aufweist.

## Revendications

1. Une composition lubrifiante liquide comprenant des hydrocarbures en C₃₀-C₁₃₀₀, ladite composition ayant un rapport de ramification compris entre 0,1 et 0,16, un poids moléculaire moyen en poids compris entre 300 et 45 000, un poids moléculaire moyen en nombre compris entre 300 et 18 000, une distribution de poids moléculaires comprise entre 1 et 5 et un point de coulée inférieur à -15°C.

2. Une composition selon la revendication 1, caractérisée en ce que lesdits hydrocarbures comprennent des hydrocarbures en C₃₀-C₁₀₀₀ et la distribution de poids moléculaire est comprise entre 1,05 et 2,5.

3. Une composition selon la revendication 1, caractérisée en ce que lesdits hydrocarbures comprennent des alcanes ou des alcènes.

4. Une composition selon la revendication 1, ayant un indice de viscosité supérieur à 130 et une viscosité à 100°C comprise entre 3 mm₂/s et 750 mm²/s.

5. Une composition selon la revendication 1, comportant une fraction en C₃₀, un indice de viscosité supérieur à 130 et un point de coulée inférieur à -45°C.

6. Une composition selon la revendication 1, caractérisée en ce que la composition comprend le résidu polymérique de 1-alcènes obtenu à partir de 1-alcènes linéaires en C₆-C₂₀.

7. Une composition selon la revendication 6, caractérisée en ce que lesdits 1-alcènes comprennent des alcènes en C₈-C₁₂.

8. Une composition selon la revendication 6, caractérisée en ce que ledit résidu polymérique comprend un résidu polymérique desdits 1-alcènes.

9. Une composition selon la revendication 6, caractérisée en ce que ledit résidu polymérique comprend du poly-1-décène.

10. Une composition selon la revendication 9, caractérisée en ce que le résidu polymérique de 1-décène a un poids moléculaire d'environ 422.

11. Une composition selon la revendication 10, ayant un indice de viscosité d'environ 134 et un point de coulée et un point de coulée inférieur à -45°C.

12. Une composition lubrifiante liquide à base d'hydrocarbure ayant une structure polymérique récurrente: dans laquelle:
n est compris entre 3 et 17, et
x est compris entre 5 et 500.

13. Une composition selon la revendication 12, dans laquelle n est égal à 7 et x moyen est au moins égal à 15.

14. Une composition selon la revendication 12, ayant un indice de viscosité supérieur à 130 et un point de coulée inférieur à -15°C.

15. Une composition d'hydrocarbure selon l'une quelconque des revendications précédentes, caractérisée en ce que les hydrocarbures en C₃₀-C₁₃₀₀ comprennent 9-méthyl,11-octylhéneicosane et 11-octyldocosane.

16. Une composition selon la revendication 15, caractérisée en ce que le rapport molaire 9-méthyl-11-octylhéneicosane/11-octyldocotane est compris entre 1/10 et 10/1.

17. Une composition selon la revendication 16, caractérisée en ce que ce rapport molaire est de préférence compris entre 1/2 et 2/1.

18. Une composition selon la revendication 15, caractérisée en ce que le 11-octyldocosane est représenté par la structure:

19. Un procédé de préparation d'hydrocarbures liquides susceptible d'être employées en tant que matières premières de lubrifiants à base d'alpha-oléfines contenant entre 6 et 20 atomes de carbone ou des mélanges de ces oléfines comprenant la mise en contact desdites oléfines dans les conditions d'oligomérisation à une température réactionnelle comprise entre 90 et 250°C avec un catalyseur de chrome fixé sur un support poreux, le catalyseur ayant été traité par oxydation à une température comprise entre 200 et 900°C en présence d'un gaz oxydant, puis il est traité par un agent réducteur à une température et pendant un temps suffisant pour réduire ledit catalyseur à un état de valence inférieure; pour obtenir une composition lubrifiante liquide oligomérique comprenant des hydrocarbures en C₃₀-C₁₃₀₀, ladite composition ayant un rapport de ramification compris entre 0,1 et 0,16, un poids moléculaire moyen en poids compris entre 300 et 45 000, un poids moléculaire moyen en nombre compris entre 300 et 18 000, une distribution de poids moléculaire comprise entre 1 et 5 et un point de coulée inférieur à -15°C.

20. Un procédé selon la revendication 19, caractérisé en ce que l'agent réducteur comprend du CO, la température d'oligomérisation est comprise entre environ 100 et 180°C et le rendement en oligomère en C₃₀⁺ est d'au moins 85% en poids pour le produit ayant une viscosité d'au moins 15 mm²/s à 100°C.

21. Un procédé selon la revendication 19 ou 20, caractérisé en ce que le support comprend de la silice poreuse.

22. Un procédé selon la revendication 19, 20 ou 21, caractérisé en ce que l'oléfine consiste essentiellement en 1-octène, 1-décène, 1-dodécène, 1-tétradécène ou les mélanges de ces composés.

23. Un procédé selon la revendication 19, 20 ou 21, caractérisé en ce que ledit catalyseur n'est pas soumis à une étape d'oxydation supplémentaire après ladite réduction.

24. Un procédé selon la revendication 19, 20 ou 21, caractérisé en ce que ladite oléfine comprend du 1-décène et l'oligomère présente un VI supérieur ou égal à 181 et un rapport de ramification compris entre 0,14 et 0,16.
